# EUROPEAN PATENT SPECIFICATION

(11) **EP 1 378 578 B1**
(45) Date of publication and mention of the grant of the patent: **07.11.2007**
(21) Application number: 02253902.7
(22) Date of filing: 05.06.2002
(51) Int. Cl.: C22C 19/00, C22C 19/05

(54) **Free-cutting Ni-base heat-resistant alloy**
Hochtemperaturfeste Nickelbasislegierung mit guter Zerspannbarkeit
Alliage de nickel résistant à des températures élevées facilement usinable

(43) Date of publication of application: 07.01.2004
(73) Proprietor: Ishida, Kiyohito, Sendai-shi, Miyagi-ken (JP); Dokuritsu Gyousei Houjin Sangyo Gijutsu Sougo Kenkyusho, Tokyo (JP); Daido Tokushuko Kabushiki Kaisha, Naka-ku Nagoya-shi Aichi-ken (JP); Tohoku Tokushuko Kabushiki Kaisha, Shibata-gun, Miyagi (JP)
(72) Inventor: Ishida, Kiyohito, Sendai-shi, Miyagi (JP); Oikawa, Katsunari, Shibata-gun, Miyagi (JP); Ueta, Shigeki, c/o Daido Tokushuko KK Gijutsu, Nagoya-shi, Aichi (JP); Noda, Toshiharu, c/o Daido Tokushuko KK Gijutsu, Nagoya-shi, Aichi (JP); Ebata, Takashi, c/o Tohoku Tokushuko KK, Shibata-gun, Miyagi (JP)
(74) Representative: Harding, Richard Patrick

(56) References cited:
- EP-A- 1 085 105
- DE-A- 4 436 670
- JP-A- 53 026 220
- PATENT ABSTRACTS OF JAPAN vol. 017, no. 025 (C-1017), 18 January 1993 (1993-01-18) & JP 04 246155 A (TOUHOKU TOKUSHIYUKOU KK), 2 September 1992 (1992-09-02)

## Description

The present invention relates to a free-cutting Ni-base heat-resistant alloy having excellent machinability.

Excellent high temperature strength is required for exhaust valves and bolts for engines since they are used under high temperature environmental conditions. There is an additional requirement for corrosion resistance against exhaust gas for exhaust pipes and valves in chemical plants as well as the requirement for high temperature strength. It has thus been a general practice to use, as a structural material for composing such parts, nickel (Ni)-base heat-resistant alloys having excellent strength and corrosion resistance in high temperature ranges.

The problem of poor machinability has, however, remained in the conventional Ni-base heat-resistant alloy, in spite of excellent strength and corrosion resistance. The machinability of structural steel or stainless steel is successfully improved by adding so-called machinability improving elements such as Pb, Bi, S, Se or Te, but the hot workability of the Ni-base heat-resistant alloy is compromised by containing such machinability improving elements. Accordingly almost no has attempts have been made to intentionally improve the machinability of Ni-base heat-resistant alloy, which has inevitably pushed up machining costs of such material in production. Fe-based and Ni-based alloys having good machinability are described in document EP 1 085 105.

It is therefore an object of the present invention to provide free-cutting Ni-base heat-resistant alloys of good strength and corrosion resistance at high temperature and in good machinability.

According to the present invention there is provided a free-cutting Ni-base heat-resistant alloy consisting of:
C in an amount of from 0.01 to 0.3 wt% and Cr in an amount of from 14 to 35 wt%;
and at least one element selected from Ti, Zr and Hf in a total amount of from 0.1 to 6 wt%, and S in an amount of from 0.015 to 0.5 wt%;
and having dispersed in the matrix thereof a machinability improving compound phase, said phase containing any one of Ti, Zr and Hf as a major constituent of the metal elements, essentially containing C and S as a binding component for such metal elements; and
satisfying the relationships: ${W}_{Ti} + 0.53 ⁢ {W}_{Zr} + 0.27 ⁢ {W}_{Hf} > 2 ⁢ {W}_{C} + 0.75 ⁢ {W}_{S} ;$
   and ${W}_{C} > 0.37 ⁢ {W}_{S}$
   where W_{Ti} represents any Ti content (wt%), W_{Zr} represents any Zr content (wt%), W_{Hf} represents any Hf content (wt%), W_{C} represents the C content (wt%) and W_{S} represents the S content (wt%) ;
and the balance being Ni in an amount of from 50 to 85 wt% and Al in an amount of from 0.1 to 5 wt%, and any inevitable impurities;
and optionally further incorporating Si in an amount of 4 wt% or less and Mn in an amount of 1 wt% or less;
and optionally further incorporating at least one of from 0.1 to 20 wt% of Co, from 0.1 to 20 wt% of Mo and from 0.1 to 20 wt% of W;
and optionally further incorporating Fe in an amount of 20 wt% or less;
and optionally further incorporating Cu in an amount of from 0.1 to 5 wt%;
and optionally further incorporating Nb and Ta in a total amount of from 0.1 to 7 wt%;
and optionally further incorporating B in an amount of from 0.0005 to 0.01 wt%;
and optionally further incorporating Se in an amount of from 0.0005 to 0.01 wt%.

By containing at least one of Ti, Zr and Hf, together with C, Cr and Al, and also with either S or Se, the Ni-base heat-resistant alloy will have generated in the matrix thereof a compound (machinability improving compound phase) based on such composition. The present inventors have found that the machinability of the Ni-base heat-resistant alloy was significantly improved by having generated in the matrix thereof such a machinability improving compound phase, which led to the present invention.

A reason why the machinability of the Ni-base heat-resistant alloy can be improved by the formation of such a machinability improving compound phase is considered to be as follows. When the alloy is subjected to processing, such as cutting or grinding, in order to remove a portion thereof, the machinability improving compound phase finely dispersed in the matrix can act just like a perforation to thereby facilitate formation of the sectional plane, which is supposed to be responsible for the improved machinability. In any event, the machinability improving compound phase can be responsible for a machinability equivalent to or superior to that attainable by the foregoing machinability improving elements previously been used, while successfully avoiding degradation of other characteristics inherent in the heat-resistant alloy and retaining good hot workability.

In the conventional Ni-base heat-resistant alloy, it has been considered necessary to intentionally control the content of sulfur (S) in order to keep good hot workability, and in some cases an effort has even been made to use a high-purity Ni material containing almost no S. By contrast, in the case of the present invention, the S content can be in an allowable range since the S will be incorporated into such machinability improving compound phase as one constituent thereof. It follows that S contained in the Ni-base heat-resistant alloy of the present invention will not heavily affect the hot workability of the alloy. This makes it possible to use a source material containing a relatively large amount of S, which is expected to result in an improved productivity.

A reason as to why the hot workability of the conventional Ni-base heat-resistant alloy is degraded by the addition of S can be explained by the formation of a (Ni, S) compound, in particular Ni₃S₂ in the alloy. In the case of the present invention, S contained in the alloy is incorporated into the machinability improving compound phase during the growth thereof, which suppresses the formation of Ni₃S₂ and thus successfully prevents the hot workability from being degraded by its S content.

Another advantage of the formation of the machinability improving compound phase is that it hardly affects the strength and corrosion resistance at high temperature, which are properties that are particularly critical for the Ni-base heat-resistant alloy. In this case, properties such as strength and corrosion resistance at high temperature are defined by residual constituents in the matrix other than such machinability improving compound phase. It follows that a heat-resistant alloy can be obtained with the desired properties by properly adjusting the composition of the matrix other than the machinability improving compound phase.

In the Ni-base heat-resistant alloy of the present invention, the machinability improving compound phase can be generated so as to be dispersed within the matrix. In particular, finer dispersion of such compound phase within the matrix will result in better machinability of the Ni-base heat-resistant alloy. In order to increase the improving effect of the machinability, it is preferable to control the average size of the machinability improving compound phase observed in the polished sectional microstructure of the Ni-base heat-resistant alloy (maximum width between two parallel tangential lines drawn in different directions so as to circumscribe the outer contour of the compound grain) within a range from 1 to 5 µm or thereabouts.

The area ratio of the machinability improving compound phase observed in a polished surface of the material is preferably 0.1 to 10%. For the purpose of obtaining an improvement in the machinability by forming such machinability improving compound phase, such phase must be contained in an amount of 0.1% or more in terms of the area ratio in the polished sectional microstructure. An excessively large area ratio will however be no more effective due to saturation of such effect, or may rather adversely affect other characteristics inherent to the heat-resistant alloy (i.e., strength and corrosion resistance at high temperature ranges). Accordingly the area ratio in the polished sectional microstructure of the Ni-base heat-resistant alloy is preferably set to 10% or below.

The machinability improving compound phase typically mainly comprises a compound expressed by a composition formula M₄Q₂C₂ (where M represents the metal element containing any one of Ti, Zr and Hf as a major constituent, and Q represents either S or Se). It is to be noted that in this specification the compound expressed by such formula may be abbreviated as "TICS". The compound has a good dispersion property into the matrix, and is particularly good at increasing the machinability.

As for the component M in the compound, it is preferable that Ti is essentially incorporated, where Zr and/or Hf may optionally be incorporated. In the case where V, Nb or Ta is incorporated in the Ni-base heat-resistant alloy, at least a part of which may compose such component M. As for the component Q, it is preferable that S is essentially incorporated, Se being optionally incorporated so as to substitute for a part of S. Both components M and Q are not precluded from incorporating any components other than those described in the above as subsidiary components in order to obtain the effect of the present invention in so far as the properties to be possessed by the machinability improving compound phase (improving machinability and good dispersion property) are not compromised thereby. The machinability improving compound phase including V, Nb, Ta or the like may possibly improve the strength of such compound.

The M₄Q₂C₂-base compound in the Ni-base heat-resistant alloy can be identified by X-ray diffractometry and electron probe X-ray micro-analysis (EPMA). For example, the presence or absence of the M₄Q₂C₂-base compound can be confirmed based on the presence or absence of the corresponding peak ascribable to such compound in a measured profile obtained by X-ray diffractometry. An area where the compound is formed in the alloy can be specified by subjecting the sectional microstructure of the alloy to surface analysis based on EPMA, and then comparing two-dimensional mapping results of characteristic X-ray intensity ascribable to Ti, Zr, Hf, S, Se or C.

The following paragraphs will describe causes for specifying ranges of contents of the individual components in the Ni-base heat-resistant alloy of the present invention.

### (1) Ni: contained as a major component

Ni is an essential component for composing the Ni-base heat-resistant alloy of the present invention, so that it is incorporated as a major component. Considering the balance with other essential additional element components, the upper limit of the content thereof is set at 85 wt%. The Ni content does not exceed 85 wt% also in the most of generally available Ni-base heat-resistant alloys, since the content exceeding 85 wt% may sometimes fail in fully demonstrating the properties specific to heat-resistant alloys due to relative shortage of contents of the residual components. So that the Ni content is preferably 85 wt% at most, and more preferably 50 to 80 wt%.

### (2) C: 0.01 to 0.3 wt%

C is an essential element for improving the machinability in the present invention. C, in coexistence with (Ti, Zr, Hr) or S described later, can form the machinability improving compound phase. The content of C less than 0.01 wt% will be too short to form the machinability improving compound phase in an amount enough for markedly improving the machinability. On the contrary, the content exceeding 0.3 wt% will increase a portion of C not contributive to the formation of the machinability improving compound phase, which will result in excessive production of other carbides and carbo-sulfides. Excessive production of such carbides and carbo-sulfides is undesirable since they are causative of degraded hot workability and ductility. The C content is more preferably 0.03 to 0.2 wt%.

### Cr: 14 to 35 wt%

Cr is an important element for ensuring corrosion resistance and oxidation resistance of the Ni-base heat-resistant alloy. Efficient achievement of such effects will be ensured in a content of 14 wt% or more. The content exceeding 35 wt% will however ruin the phase stability, which results in lowered toughness and degraded anti-oxidative property. The Cr content is more preferably set within a range from 16 to 30 wt%, and still more preferably from 18 to 25 wt%.

### (4) At least one of (Ti, Zr, Hf) in a total amount of 0.1 to 6 wt%

Ti, Zr or Hf is an essential component element of the machinability improving compound phase which plays a principal role in exhibiting improving effect of the machinability of the free-cutting Ni-base heat-resistant alloy of the present invention. The total content of at least one of these elements of less than 0.1 wt% will result in an insufficient amount of production of the machinability improving compound phase, so that a sufficient improving effect of the machinability cannot be expected. On the contrary, when the total amount is excessive, (Ti, Zr, Hf) may form compounds with other elements to thereby lower the machinability. So that the total content of these elements is necessarily suppressed to 6 wt% or less. A part of (Ti, Zr, Hf) as the metal component elements composing the machinability improving compound phase may be substituted by Nb or Ta, which elements can contribute to the formation of γ' phase to thereby improve the high-temperature strength of the Ni-base heat-resistant alloys. Zr and Hf are not so much effective in improving the machinability and high-temperature strength as compared with Ti, so that of these elements, it is more preferable to employ Ti as a major component. In this case the Ti content is preferably set within a range from 0.1 to 4 wt% in order to efficiently obtain such effect. Although Zr and Hf are not so effective as Ti in improving the machinability and high-temperature strength cf the alloy, they are advantageous in raising the grain boundary strength through segregation within the grain boundary, so that they may be contained to an extent not causative of attenuating the Ti-related benefit. It is to be noted that composing the metal component of the machinability improving compound phase only with Zr and/or Hf can also be effective in improving the machinability and high-temperature strength.

### (5) S: 0.015 to 0.5 wt%

S is an effective element for improving the machinability. By containing S, compounds effective for raising the machinability (e.g., the foregoing machinability improving compound phase) can be formed within the alloy texture. So that the lower limit of the S content is defined as 0.015 wt%. Excessive addition of S will however increase a portion of S not involved in the formation of the machinability improving compound phase (referred to as "free S"), which eventually promote the formation of (Ni, S) compounds, in particular Ni₃S₂ causative of degrading the hot workability. While the amount of formation of the machinability improving compound phase increases with the S content, excessive formation thereof will degrade properties specific to the heat-resistant alloy. So that the upper limit of the S content is defined as 0.5 wt%. To obtain the improving effect of the machinability by such compound to a desirable degree, it is preferable to properly adjust the S content according to Lhe amount of addition of other constituents of the machinability improving compound phase such as C, Ti, Zr, Hf or so. The free S is preferably as less as possible, and it is desirable to adjust the S content so that almost all portion of S added to the Ni-base heat-resistant alloy will compose the machinability improving compound phase.

The component Q other than S (which herein means Se) may be included in the machinability improving compound phase so as to substitute for S composing such phase. In this case, the Se content is preferably set within a range from 0.0005 to 0.1 wt%. The content less than 0.0005 wt% will be meaningless since the effect of the addition will hardly become clear. On the other hand, the content exceeding 0.1 wt% may sometimes degrade the hot workability and other properties specific to the heat-resistant alloy.

### (6) Satisfying relations of:

${W}_{Ti} + 0.53 ⁢ {W}_{Zr} + 0.27 ⁢ {W}_{Hf} > 2 ⁢ {W}_{C} + 0.75 ⁢ {W}_{S} ;$
and ${W}_{C} > 0.37 ⁢ {W}_{S}$
where W_{Ti} represents Ti content (wt%), W_{Zr} represents 2r content (wt%), W_{Hf} represents Hf content (wt%), W_{C} represents C content (wt%) and W_{S} represents S content (wt%).
The left side of the formula A represents a parameter reflecting the total number of (Ti, Zr, Hf) atoms. That is, the foregoing machinability improving effect by the machinability improving compound phase is determined based on the total number of atoms (or the molar number), not on the total weight of the constituents to be included. Also the right side of the formula **A** represents a parameter reflecting the total number of (C, S) atoms. Coefficients for W_{Ti}, W_{Zr}, and W_{Hf} appear on the left side of the formula A are determined based on a fact that ratio of the number of (Ti, Zr, Hf) atoms per unit weight of the alloy is round to be 1:0.53:0.27, and similarly, coefficients for W_{c} and Wₛ appear on the right side of the formula A are determined based on a fact that ratio of the number of (C, S) atoms per unit weight of the alloy is found to be 2:0.75. So that it is to be understood that the formula **A** is such that comparing the total numbers of (Ti, Zr, Hf) atoms and (C, S) atoms. Similarly, the formula **B** can be understood as a formula for comparing the numbers of C and S atoms contained in the alloy.

Assuming that all parts of (Ti, Zr, Hf, C, S) atoms added to the alloy are to be involved for the formation of TICS expressed by formula M₄Q₂C₂, satisfying the above formula **A** expressing (left side) > (right side) will inevitably mean that a portion of (Ti, Zr, Hf) atoms not contributing to the formation of TICS can remain in the residual alloy part. Such portions of (Ti, Zr, Hf) will however hardly affect the properties of the heat-resistant alloy even they remain in the residual alloy part to some extent, or rather, they may compose the γ' phase to thereby raise the strength. On the contrary in the case of (left side) < (right side), a portion of at least either of (C, S) atoms will never contribute to the formation of TICS and remain in the residual alloy part in a free form. Free S remaining in the residual alloy part is undesirable since it may react with Ni to thereby form (Ni, S) compound, in particular Ni₃S₂, causative of degrading the hot workability. On the other hand, C which is present in the residual alloy part other than the machinability improving compound phase may degrade the machinability or properties specific to the heat-resistant alloy due to promoted formation of carbides other than such machinability improving compound. Thus the formula **A** is necessarily be satisfied.

Further satisfying herein the formula **B** ensures that the number of S atoms to be contained is smaller than that of C. This ensures that S to be contained will almost completely be fixed to the machinability improving compound phase, and will suppress the content of free S residing in the matrix other than such machinability improving compound phase. A portion of C not involved in the formation of the machinability improving compound phase may sometimes result in the formation of carbides responsible for raising the creep strength. This is why the formula **B** is defined at least as (left side) > (right side). However as has been described in the above, excessive free C may degrade the machinability or other properties of the alloy, so that it is more preferable to satisfy the following formula: $0.37 ⁢ {W}_{S} + 0.1 > {W}_{C}$
in order to suppress the excessive free C.

In the free-cutting Ni-base heat-resistant alloy of the present invention, the Si content is preferably set to 4 wt% or less, and Mn to 1 wt% or less.

### (7) Si : 4 wt% or less

Si is inevitably contained in the alloy as a deoxidizing element. Intentional addition thereof to a certain extent will be also allowable since the element has an improving effect of the oxidation resistance of the Ni-base heat-resistant alloy. To obtain the oxidation resistance to a sufficient degree, the addition in an amount of at least 0.1 wt% is recommendable. It is also recommendable to suppress the content to 4 wt% or less since excessive content thereof will degrade the hot workability and ductility

### Mn: 1 wt% or less

Mn is inevitably contained in the alloy as a deoxidizing element. Excessive content thereof however is not desirable since it may not only degrade the corrosion resistance but also promote the deposition of Ni₃Ti which is a phase responsible for embrittlement. So that the content thereof is preferably suppressed to 1 wt% or less.

The alloy of the present invention may further contain 0.1 to 5 wt% of Al in order to improve the high-temperature strength and corrosion resistance.

### (9) Al: 0.1 to 5 wt%

In the Ni-base heat-resistant alloy, Al is responsible for solid solution hardening by forming solid solution in the matrix thereof, or for precipitation hardening of γ' phase by forming γ' phase (Ni₃Al) by reacting with the Ni component. Al which can form solid solution in the alloy is also expectable for its effect of improving the oxidation resistance at high temperature ranges. The high-temperature strength of the Ni-base heat-resistant alloy is often largely contributed especially by precipitation hardening of such γ' phase formation. So that the Al content within the above range is preferable in view of obtaining desirable properties specific to the heat-resistant alloy. Al content of less than 0.1 wt% results in the foregoing effect only to an insufficient degree. On the other hand, the content exceeding 5 wt% will inhibit the hot working, so that the Al content is more preferably set within a range from 0.2 to 3 wt%.

The Ni-base heat-resistant alloy of the present invention can contain at least any one of 0.1 to 20 wt% of Co, 0.1 to 20 wt% of Mo and 0.1 to 20 wt% of W.

### (10) Co: 0.1 to 20 wt%

Similarly to Ni, Co can stabilize the austenitic phase, and increases the amount of formation of the γ' phase, which is a precipitation hardening phase, to thereby improve the strength of the alloy. Co may sometimes improve the high-temperature strength of the alloy by forming solid solution in the Ni component. To obtain the effect of addition to a desirable degree, the Co content is preferably set to 0.1 wt% or above. On the other hand, the addition exceeding 20 wt% is no more desirable since the effect of solid solution hardening will saturate, and the cost will increase.

### (11) Mo: 0.1 to 20 wt%; W: 0.1 to 20 wt%

Mo and W are responsible for improving high-temperature strength of the alloy by forming solid solution in the texture thereof, and for improving corrosion resistance based on passivation enhancement. The contents less than 0.1 wt% will fail in obtaining a sufficient effect, and on the contrary exceeding 20 wt% will undesirably ruin the hot workability of the alloy.

It is further preferable in the present invention to suppress the Fe content to 20 wt% or less. Fe is often used as the basic component of the Ni-base heat-resistant alloy as well as Ni and Cr, but this is largely because Fe is relatively easy to handle and inexpensive. Increasing the Fe content while making a great account of cost has however degraded the corrosion resistance of the Ni-base heat-resistant alloy due to relative decrease in the Ni and Cr contents. So that for the applications in which the corrosion resistance is of a great importance, the Fe content is preferably suppressed to 20 wt% or less. Further, the Fe content is preferably suppressed to 10 wt% or less and more preferably 5 wt% or less.

The Ni-base heat-resistant alloy of the present invention may also contain 0.1 to 5 wt% of Cu. Cu is advantageous in improving the corrosion resistance, in particular that in the reductive acidic environment (in particular sulfuric acid environment), and also in reducing the work hardening property to thereby improve the workability. Cu can also be added in order to improve the antibacterial property, which can be enhanced by annealing. The Cu content is necessarily set to 0.1 wt% or above to ensure such effects. The excessive addition however degrades the hot workability, so that the content is preferably set within a range of 5 wt% or below.

The Ni-base heat-resistant alloy of the present invention may also contain Nb and Ta in a total amount of 0.1 to 7 wt%. Such components added to the alloy will form solid solution in the γ' phase (Ni₃Al) formed in the texture of the Ni-base heat-resistant alloy, to thereby raise the strength of such γ' phase (Ni₃Al), and thus raise the high-temperature strength of the entire alloy. Such components can also be included in the foregoing machinability improving compound phase to thereby increase the strength thereof. To obtain such effect to a desirable extent, the total content thereof is preferably set to 0.1 wt% or above. On the contrary, the content exceeding 7 wt% will undesirably degrade the toughness. More preferable total amount of Nb and Ta resides within a range from 0.5 to 5 wt%.

The Ni-base heat-resistant alloy of the present invention may also contain 0.0005 to 0.01 wt% of B. B is a valuable element for improving the hot workability. The content less than 0.0005 wt% will result in only a limited range of effects, and exceeding 0.01 wt% will degrade the hot workability.

Specific examples of materials applicable to the Ni-base heat-resistant alloy of the present invention will be listed below (all in trade names). It is to be defined that the alloy compositions thereof are such that containing machinability improving elements (Ti, Zr, Hf, S, Se, C, etc.) specified in the present invention so as to substitute for a part of Ni as a major component. So that, the names listed below mean specific alloys of the present invention derived from the alloys whose composition are specified by the product standard, although the product names were quoted herein for convenience. Individual alloy compositions of the original products are described in "Kinzoku Deta Bukku (Metal Data Book), 3rd edition.", p. 138, published by Maruzen, and will not be detailed in this specification.
(1) Solution-hardened Ni-base heat-resistant alloy: Hastelloy-C22, Hastelloy-C276, Hastelloy-G30, Hastelloy X, Inconel 600 and KSN.
(2) Precipitation-hardening Ni-base heat-resistant alloy: Astroloy, Cabot 214, D-979, Hastelloy S, Hastelloy XR, Haynes 230, Inconel 587, Inconel 597, Inconel 601, Inconel 617, Inconel 625, Inconel 706, Inconel 718, Inconel X750, M-252. Nimonic 75, Nimonic 30A, Nimonic 90, Nimonic 105, Nimonic 115, Nimonic 263, Nimonic PE-11, Nimonic PE. 16, Nimonic PK.33, Rene 41, Rene 95, SSS 113MA, Udimet 400, Udimet 500, Udimet 520, Udimet 630, Udiment 700, Udimet 710, Udimet 720, Unitemp AF 2-1 DA 6 and Waspaloy.

### DETAILED DESCRIPTION OF THE PREFERRED EMBODIMENTS

### (Examples)

The following experiments were carried out to investigate the effects of the present invention.

The individual alloys of the present invention and comparative alloys respectively having compositions listed in Tables 1 and 2 were melted in a vacuum induction heater to thereby obtain 50-kg alloy ingots. The ingots were then kept at 1,200°C for homogenization, and were then processed by hot forging within a temperature range from 1,200 to 1,000°C to thereby obtain round rods of 65 mm in diameter. A part of such rods was further forged to reduce the diameter to as small as 20 mm. The rods were then subjected to solution heat treatment at 1,100°C for 1 hour, and then successively to age hardening at 700°C for 16 hours. The 65-mm-diameter rods were subjected to machinability evaluation, and the 20-mm-diameter rods were subjected to evaluation of hot workability , hardness after aging and creep characteristics.

While a major inclusion in the alloy of the present invention was found to be a compound expressed as (Ti, Zr, Hf)₄S₂C₂ (TICS), some alloys were also found to include (Ti, Zr, Hf)-base sulfide such as (Ti, Zr, Hf)S, or (Ti, Zr, Hf)-base carbide such as (Ti, Zr, Hf)C. There was almost no sign of presence of Ni-S compounds, in particular Ni₃S₂, in the Ni-base heat-resistant alloy of the present invention.

Such inclusions were identified by the following procedure. Each round rod was cut to produce a proper amount of test pieces, and the metal matrix thereof was dissolved by an electrolytic process using a methanol solution containing tetramethylammonium chloride and 10% actylacetone as an electrolyte. The electrolytic solution after the solubilization was filtered to thereby extract the insoluble compound contained in the Ni-base alloy. The extracted compound was dried, and was then analyzed by X-ray diffractometry for identification based on observed peaks in the diffraction profile. The composition of the compound grains in the alloy was separately analyzed by EPMA. A two-dimensional mapping based on the EPMA analysis proved formation of a compound having a composition corresponded to that of a compound identified by the X-ray diffractometry.

The individual test pieces were then subjected to each of the following experiments.

### 1. Machinability Test

Machinability was evaluated based on the amount of wear of the tool when the test piece was cut, and on roughness of the cut surface. A machining tool employed was made of a cemented carbide, with which wet cutting was performed at a peripheral speed of 30 m/min, feed per revolution of 0.2 mm, and depth of cut per revolution of 1.5 mm. The amount of wear of the tool was defined by flank wear on the machining tool after 30 minutes of cutting. Roughness of the cut surface was obtained by measuring arithmetical mean (Ra: µm) of the sample surface after the cutting based on JIS-B0601.

### 2. Hot Workability Evaluation

A test piece of 6 mm in diameter was cut from the 20-mm-diameter rod, and then subjected to tensile test to thereby evaluate the hot workability. The test was performed using a high-speed tension tester at various temperatures from 900 to 1,250°C, and tensile speed of 50 mm/sec. Defining now the hot workable range as a temperature range in which rupture drawing of not less than 40%, which is a required value for allowing forging, is ensured, the samples having such temperature range of 200°C or more were assessed as "excellent in hot workability (○)", and those having such temperature range of less than 200°C were assessed as "poor in hot workability (×)".

### 3. Hardness Test

C-scale Rockwell hardness of the Ni-base heat-resistant alloy was measured at room temperature according to the Rockwell hardness testing procedures specified in JIS-Z2245.

### 4. High-Temperature Strength Evaluation

The high-temperature strength was evaluated by carrying out creep rupture test based on the method specified by JIS-Z2272. More specifically, a test piece of 6 mm in diameter was cut from the 20-mm-diameter rod, and then subjected to creep test at 700°C under a 400-MPa load, and the duration of time before the test piece ruptures was measured.

Experimental results of these tests were shown together in Table 3.

**Table 3**

| No. | Cutting Test | | Hot workability Temperature range ensuring 40% or more drawing of 200°C or above | Hardness after aging (HRC) | Creep rupture time (hr) |
|---|---|---|---|---|---|
| | Flank wear (*µ*m) | Roughness of cut surface (µm) | | | |
| 1 | 183 | 3.8 | ○ | 37.8 | 287 |
| 2 | 132 | 3.4 | ○ | 32.3 | 141 |
| 3 | 178 | 3.4 | ○ | 30.1 | 93 |
| 4 | 167 | 3.2 | ○ | 38.4 | 304 |
| 5 | 154 | 3.0 | ○ | 33.0 | 150 |
| 6 | 124 | 3.5 | ○ | 41.6 | 342 |
| 7 | 149 | 3.1 | ○ | 38.2 | 295 |
| 8 | 131 | 3.3 | ○ | 32.5 | 149 |
| 9 | 170 | 3.4 | ○ | 35.3 | 216 |
| 10 | 165 | 3.2 | ○ | 39.1 | 324 |
| 11 | 196 | 3.4 | ○ | 44.9 | 418 |
| 12 | 312 | 8.2 | ○ | 37.4 | 278 |
| 13 | 299 | 7.8 | ○ | 32.1 | 134 |
| 14 | 186 | 3.4 | × | 30.3 | 89 |
| 15 | 238 | 8.4 | × | 37.9 | 208 |
| 16 | 197 | 3.7 | × | 33.2 | 143 |
| 17 | 225 | 4.3 | × | 26.8 | 75 |
| 18 | 257 | 4.6 | × | 30.7 | 97 |
| 19 | 155 | 3.5 | × | 41.6 | 241 |
| 20 | 191 | 3.8 | ○ | 38.9 | 106 |
| 21 | 231 | 5.4 | × | 50.3 | 332 |
| 22 | 189 | 3.9 | × | 40.1 | 223 |
| 23 | 143 | 3.2 | ○ | 39.4 | 188 |
| 24 | 136 | 3.2 | ○ | 20.8 | 44 |
| 25 | 192 | 4 | × | 44.5 | 256 |

It was made clear from Table 3 that the Ni-base heat-resistant alloy of the present invention in Examples 1 to 11 showed excellent hardness after aging at room temperature and creep characteristics at high temperature ranges, which proved satisfactory characteristics specific to the heat-resistant alloy, and excellent machinability as well. On the contrary, Comparative Examples 12 and 13 showed only poor machinability, which was ascribable to insufficient formation of TICS, which is the machinability improving compound phase, due to an extremely low S content. Comparative Example 14 showed an excellent machinability by the formation of TICS, but was found to be poor in the hot workability due to an excessive S content. Comparative Example 15 showed an excellent creep characteristic at a high temperature range, but was found to be poor in the machinability and hot workability due to an excessive C content. Comparative Example 18 showed only a poor machinability, which was ascribable to insufficient formation of TICS due to an extremely low total contents (M) of (Ti, Zr, Hf), and was found also poor in the hot workability since S cannot be fixed by TICS. Comparative Example 19 showed only a poor hot workability due to excessive M.

It was thus concluded that the Ni-base heat-resistant alloy of the present invention can successfully improve the machinability without ruining the hot workability, while retaining the other characteristics specific to the heat-resistant alloy as comparable to those of the conventional heat-resistant alloys.

## Claims

1. A free-cutting Ni-base heat-resistant alloy consisting of:
C in an amount of from 0.01 to 0.3 wt% and Cr in an amount of from 14 to 35 wt%;
and at least one element selected from Ti, Zr and Hf in a total amount of from 0.1 to 6 wt%, and S in an amount of from 0.015 to 0.5 wt%;
and having dispersed in the matrix thereof a machinability improving compound phase, said phase containing any one of Ti, Zr and Hf as a major constituent of the metal elements, essentially containing C and S as a binding component for such metal elements; and
satisfying the relationships: ${W}_{Ti} + 0.53 ⁢ {W}_{Zr} + 0.27 ⁢ {W}_{Hf} > 2 ⁢ {W}_{C} + 0.75 ⁢ {W}_{S} ;$
and ${W}_{C} > 0.37 ⁢ {W}_{S}$
where W_{Ti} represents any Ti content (wt%), W_{Zr} represents any Zr content (wt%), W_{Hf} represents any Hf content (wt%), W_{C} represents the C content (wt%) and W_{S} represents the S content (wt%) ;
and the balance being Ni in an amount of from 50 to 85 wt% and Al in an amount of from 0.1 to 5 wt%, and any inevitable impurities;
and optionally further incorporating Si in an amount of 4 wt% or less and Mn in an amount of 1 wt% or less;
and optionally further incorporating at least one of from 0.1 to 20 wt% of Co, from 0.1 to 20 wt% of Mo and from 0.1 to 20 wt% of W;
and optionally further incorporating Fe in an amount of 20 wt% or less;
and optionally further incorporating Cu in an amount of from 0.1 to 5 wt% ;
and optionally further incorporating Nb and Ta in a total amount of from 0.1 to 7 wt%;
and optionally further incorporating B in an amount of from 0.0005 to 0.01 wt%
and optionally further incorporating Se in an amount of from 0.0005 to 0.1 wt%.

2. The free-cutting Ni-base heat-resistant alloy according to Claim 1, wherein said machinability improving compound phase mainly comprises a component phase expressed by a composition formula M₄Q₂C₂ where M represents the metal element component containing Ti, Zr and/or Hf as constituents, and Q represents the component comprising S and any Se.

3. The free-cutting Ni-base heat-resistant alloy according to Claim 1 or 2, further satisfying the relationship 0.37W_{S} + 0.1 >W_{C}.

## Patentansprüche

1. Wärmebeständige Automatenlegierung auf Nickelbasis, bestehend aus:
C in einer Menge von 0,01 bis 0,3 Gewichtsprozent und Cr in einer Menge von 14 bis 35 Gewichtsprozent;
und mindestens einem Element, das ausgewählt wird unter Ti, Zr und Hf in einer Gesamtmenge von 0,1 bis 6 Gewichtsprozent sowie S in einer Menge von 0,015 bis 0,5 Gewichtsprozent;
und, mit in der Matrix derselben dispergiert, einer die Bearbeitbarkeit verbessernden Verbundphase, wobei diese Phase irgendein Element aus Ti, Zr und Hf als einen wesentlicheren Bestandteil unter den Metallelementen enthält, und zwar im Wesentlichen C und S als eine Bindungskomponente für solche Metallelemente enthaltend; und
den nachfolgenden Beziehungen entsprechend: ${W}_{Ti} + 0 , 53 {W}_{Zr} + 0 , 27 ⁢ {W}_{Hf} > 2 {W}_{C} + 0 , 75 {W}_{S} ;$
und ${W}_{C} > 0 , 37 {W}_{S}$
in welchen W_{Ti} irgendeinen Ti-Gehalt (Gewichtsprozent), W_{Zr} irgendeinen Zr-Gehalt (Gewichtsprozent), W_{Hf} irgendeinen Hf-Gehalt (Gewichtsprozent), W_{C} den C-Gehalt (Gewichtsprozent) und W_{S} den S-Gehalt (Gewichtsprozent) darstellen;
und der Rest aus Ni in einer Menge von 50 bis 85 Gewichtsprozent und aus Al in einer Menge von 0,1 bis 5 Gewichtsprozent und aus irgendwelchen unvermeidbaren Verunreinigungen besteht;
und wahlweise ferner Si in einer Menge von 4 Gewichtsprozent oder weniger und Mn in einer Menge von 1 Gewichtsprozent oder weniger enthält;
und wahlweise ferner mindestens eines aus 0,1 bis 20 Gewichtsprozent Co, 0,1 bis 20 Gewichtsprozent Mo und von 0,1 bis 20 Gewichtsprozent W enthält:
und wahlweise ferner Fe in einer Menge von 20 Gewichtsprozent oder weniger enthält;
und wahlweise ferner Cu in einer Menge von 0,1 bis 5 Gewichtsprozent enthält;
und wahlweise ferner Nb und Ta in einer Gesamtmenge von 0,1 bis 7 Gewichtsprozent enthält;
und wahlweise ferner B in einer Menge von 0,0005 bis 0,01 Gewichtsprozent enthält;
und wahlweise ferner Se in einer Menge von 0,0005 bis 0,1 Gewichtsprozent enthält;

2. Wärmebeständige Automatenlegierung auf Nickelbasis gemäß Anspruch 1, bei welcher die besagte die Bearbeitbarkeit verbessernde Verbundphase im Wesentlichen eine Komponentenphase umfasst, die ausgedrückt wird durch eine Zusammensetzungsformel M₄Q₂C₂, in welcher M die Metallelementkomponente darstellt, die Ti, Zr und / oder Hf als Stoffbestandteile enthält, und Q die Komponente darstellt, welche S and irgendein Se umfasst.

3. Wärmebeständige Automatenlegierung auf Nickelbasis gemäß Anspruch 1 oder 2, welche ferner die Beziehung 0,37 W_{S} + 0,1 > W_{C} erfüllt.

## Revendications

1. Alliage de décolletage résistant à la chaleur à base de Ni constitué:
de C dans une quantité de 0,01 à 0,3% en poids et de Cr dans une quantité de 14 à 35% en poids;
et d'au moins un élément choisi parmi Ti, Zr et Hf dans une quantité totale de 0,1 à 6% en poids, et de S dans une quantité de 0,015 à 0,5% en poids;
et présentant dispersée dans la matrice de celui-ci, une phase de composés améliorant la capacité d'usinage, ladite phase contenant l'un quelconque de Ti, Zr et Hf comme constituant majeur des éléments métalliques, contenant essentiellement C et S comme composant de liaison pour ces éléments métalliques; et
satisfaisant les relations: ${W}_{Ti} + 0 , 53 ⁢ {W}_{Zr} + 0 , 27 ⁢ {W}_{Hf} > 2 ⁢ {W}_{C} + 0 , 75 ⁢ {W}_{S} ;$
et ${W}_{C} > 0 , 37 ⁢ {W}_{S}$
où W_{Ti} représente toute teneur en Ti (% en poids), W_{Zr} représente toute teneur en Zr (% en poids), W_{Hf} représente toute teneur en Hf (% en poids), W_{c} représente la teneur en C (% en poids) et Wₛ représente la teneur en S (% en poids);
et le reste étant Ni dans une quantité de 50 à 85% en poids et Al dans une quantité de 0,1 à 5% en poids, et toutes impuretés inévitables;
et éventuellement incorporant en outre Si dans une quantité de 4% en poids ou moins et Mn dans une quantité de 1% en poids ou moins;
et éventuellement incorporant en outre au moins un parmi de 0,1 à 20% en poids de Co, de 0,1 à 20% en poids de Mo et de 0,1 à 20% en poids de W;
et éventuellement incorporant en outre Fe dans une quantité de 20% en poids ou moins;
et éventuellement incorporant en outre Cu dans une quantité de 0,1 à 5% en poids;
et éventuellement incorporant en outre Nb et Ta dans une quantité totale de 0,1 à 7% en poids;
et éventuellement incorporant en outre B dans une quantité de 0,0005 à 0,01% en poids;
et éventuellement incorporant en outre Se dans une quantité de 0,0005 à 0,1% en poids.

2. Alliage résistant à la chaleur à base de Ni de décolletage suivant la revendication 1, dans lequel ladite phase de composés améliorant la capacité d'usinage comprend principalement une phase de composants exprimée par une formule de composition M₄Q₂C₂, où M représente le composant d'élément métallique contenant Ti, Zr et/ou Hf comme constituants, et Q représente le composant contenant S et tout Se.

3. Alliage résistant à la chaleur à base de Ni de décolletage suivant la revendication 1 ou 2, satisfaisant en outre la relation 0,37W_{S} + 0,1 > W_{C}.
